

Feb. 16, 1926.

1,573,219

C. A. CADWELL

MANUFACTURE OF RAIL BONDS

Filed Jan. 18, 1922

2 Sheets-Sheet 1



Fig. 1



Fig. 2

INVENTOR,  
Charles A. Cadwell  
BY  
Fay, Oberlin & Fay  
ATTORNEY,

Feb. 16, 1926.

1,573,219

C. A. CADWELL

MANUFACTURE OF RAIL BONDS

Filed Jan. 18, 1922

2 Sheets-Sheet 2



INVENTOR  
Charles A. Cadwell  
BY  
Fay, Oberlin & Fay.  
ATTORNEYS.

## UNITED STATES PATENT OFFICE.

CHARLES A. CADWELL, OF CLEVELAND, OHIO, ASSIGNEE TO THE ELECTRIC RAIL-WAY IMPROVEMENT COMPANY, OF CLEVELAND, OHIO, A CORPORATION OF OHIO.

## MANUFACTURE OF RAIL BONDS.

Application filed January 18, 1922. Serial No. 530,133.

To all whom it may concern:

Be it known that I, CHARLES A. CADWELL, a citizen of the United States, and a resident of Cleveland, county of Cuyahoga, and State of Ohio, have invented a new and useful Improvement in the Manufacture of Rail Bonds, of which the following is a specification, the principle of the invention being herein explained and the best mode in which I have contemplated applying that principle, so as to distinguish it from other inventions.

The present invention relates more particularly to the manufacture of rail bonds of the type consisting of a flexible body portion of copper or equivalent metal of high conductivity to the terminals of which are brazed pieces of steel of relatively substantial bulk, whereby such terminals are adapted to be attached to the rail by arc welding. One form of bond having the construction just referred to is described and claimed in the co-pending application of William E. Huber and Charles A. Cadwell, filed January 18, 1922, Ser. No. 530,132, and the manufacture of such bond is shown herein as illustrating the steps of the process or details of the apparatus or mechanism of present interest.

The object of the present invention is to provide a simple and inexpensive method for manufacturing bonds of this type in the shop whereby a plurality of such bonds may be equipped with terminals of steel or equivalent metal with a minimum of effort on the part of the operator and assurance that uniformly perfect welds will be obtained between the ends of the copper conductors forming the bodies of the bonds and such terminals.

To the accomplishment of the foregoing and related ends said invention, then, consists of the means hereinafter fully described and particularly pointed out in the claims, the annexed drawings and the following description setting forth in detail certain means and one mode of carrying out the invention, such disclosed means and mode illustrating, however, but one of various ways in which the principle of the invention may be used.

In said annexed drawings:—

Fig. 1 is a side elevation with a portion sectioned away of an apparatus adapted for carrying on my present improved method

of manufacturing bonds of the type in question; Fig. 2 is a plan view of such apparatus; Fig. 3 is a transverse section thereof taken on the plane indicated by the line 3—3 on Figs. 1 and 2; Fig. 4 is a section of a detail of the apparatus taken at right angles to that in Fig. 3, as indicated by the line 4—4 on said figure; Fig. 5 is a plan view similar to that of Fig. 2 but illustrating a modification in the form of the apparatus; and Fig. 6 is a transverse section of such modified form of apparatus, the plane thereof being indicated by the line 6—6, Fig. 5.

A typical form of bond in the manufacture of which my improved apparatus is intended to be employed, as shown in Figs. 3 and 4, comprises a body 1 composed of stranded conductors of copper or equivalent highly conductive material. The respective ends of such bond body are enclosed in a sleeve 2, preferably of the same metal, such sleeve being conveniently formed by wrapping a narrow band of copper, for example, around the ends of the conductor and thereupon placing same under heavy pressure between suitable dies with the result that the component strands entering into such end are rendered practically solid. The finished bond terminal includes a piece of steel or equivalent metal which, in the particular form of bond illustrated, takes the form of a short section 3 of cylindrical rod having a diameter approximately equal to the transverse width of the preformed terminal. The latter is brazed to such rod section or piece of steel, whatever its form, by depositing around the same a suitable quantity of molten brass or equivalent brazing material and it is for the purpose of thus brazing such terminals to the ends of the bond bodies that the present apparatus has been designed.

In the illustrative form of such apparatus shown in Figs. 1 to 4, inclusive, I utilize a plurality of graphite molds 4 of general rectangular form with their ends flaring downwardly and outwardly (see Fig. 3). Each of these molds is formed with a recess 4<sup>a</sup> of just the proper length and width to receive the steel piece 3 that forms the bond terminal proper, and of a depth sufficient to include, in addition to such steel piece, the preformed end of the bond enclosed by the sleeve 2. The bond body is supported by a

suitable jig 5, or other means, with such mold or rather a similarly shaped filler block 17 by the adjacent transverse bar 12. It will accordingly be seen that the current will traverse the entire series of molds 4 in passing from one such terminal conductor 16 to the other. The molds being most conveniently made of graphite, which is a relatively good conductor of electricity, I increase the resistance of the path and cause a more intense heating of such mold by interposing thin carbon plates 18 between successive molds. If desired, a plurality of such carbon plates or laminations may be thus interposed, as shown in Fig. 4, in order to increase the resistance at these points and thus the heating effect which is conducted directly to the graphite molds. 70  
75  
80  
85  
90  
95  
100  
105  
110  
115  
120  
125  
130

suitable jig 5, or other means, with such preformed end resting on the steel piece and the mold is then raised to a high temperature as by passing a heating electric current therethrough as will be presently described. Simultaneously with such heating of the mold, braze material is fed into the recess onto the steel piece adjacent the preformed bond end. In the form of apparatus under consideration two brass rods 7, 7, are shown as being simultaneously fed into the mold, being guided in suitable tubes 8, 8, provided for this purpose, and as the ends of these rods melt off, the molten brass will fill the mold above the steel piece 3 and around the preformed end to the desired height, whereupon the operation is stopped, and as soon as the molten metal has sufficiently cooled, the bond is removed and any excess brass machined off of the terminal. As a result the steel piece whether of the rod section, shown in Figs. 3 and 4, or of other shape, is firmly united to the sleeve 2 and included strands of the material forming the body of the bond by surrounding mass 9 of brass. The body of the bond may then be bent into U or other shape, depending upon the particular use to which it is to be put, whether for connecting the immediately abutting ends of rails or for so-called crossover connections, etc.

In order to facilitate the carrying out of the brazing operation involved in forming the terminals of successive bonds, as just described above, I preferably align a plurality of molds 4 on a suitable bed 10 of heat resistant material that at the same time is a non-conductor of electricity. Two bars or blocks 11 lie on said bed 10, one on each side of the aligned series of molds, said bars having their inner faces beveled in a direction the reverse of that of the ends of the molds so as to assist in holding the latter in place. The assembled series of molds is clamped together by means of two transverse bars 12, 12, one at each end of the series, that are connected together by means of tie rods 13, 13, which are suitably insulated from the one such bar and are provided with nuts in the form of hand wheels 14 at their opposite ends that adjustably press against the corresponding bar through the medium of compression springs 15. It is the purpose of these springs to automatically maintain a nearly constant pressure on the line of blocks forming the resistance path of the heating current, since the electrical resistance of this path varies with the pressure and the pressure changes with the expansion of the materials due to heat.

Current is supplied to the respective ends of the series of molds by means of suitable electrodes or conductors 16, 16, that are clamped against the respective terminal

In operation, the steel pieces 3 that form the terminals of the bonds are placed in the bottoms of the recesses 4 in the several molds. Thereupon the preformed bonds, one or more up to the total number of the molds 4 provided in the apparatus, are disposed each with one end resting upon such terminal piece, the temperature of which along with such bond end is raised to the proper temperature for brazing by turning on the electric current and then sufficient brazed material to effectually unite the two parts in question is supplied to each such mold recess. Upon turning off the current the molds quickly cool to a point where the bonds may be removed and reversed in position to form the terminals on their opposite ends or else new bonds be substituted, as the case may be. The heating effect of the electric current can be modified to a degree by appropriately regulating the pressure upon the assembled series of graphite molds and interposed carbon laminations by turning the hand wheels 14 in one direction or the other. It will be understood that a suitable fluxing material will be added along with the brazing material in order to insure a perfect union between the component parts of the bond terminal. Indeed, the graphite and carbon blocks are preferably kept completely immersed in, and covered by, a bath of melted borax, such bath serving to keep the hot graphite and carbon from contact with the air, which would otherwise cause the same to burn away. At the same time, of course, such bath performs the function of a flux for the brazing operation. It will also be understood that the body of brass that unites the steel piece constituting the terminal proper to the end of the bond body may be machined or otherwise finished, as desired.

In the modified form of apparatus illustrated in Figs. 5 and 6, I employ a series of graphite molds 4 with interposed carbon laminations 18 as before. Instead, however, of only two tie rods, one on each side for clamping such assembled molds together, I

employ four such rods 20, two on each side, the inner ends of each pair being attached to a bracket 21 projecting laterally from the bed 10 and the outer ends of both being provided 5 with nuts in the form of hand wheels 14 that bear against the adjacent transverse bar 12 through the medium of springs 15. I also employ, instead of a jig of the type shown in Figs. 1 and 3 for holding the bond and 10 feeding the brazed material into the mold, a series of lateral stay members 22 adjustably supported upon a bar 23 disposed alongside the series of molds, the forward ends of these members serving to support between them the successive bonds which may 15 have their ends lightly concaved to insure that they will rest in proper central position over the pieces of steel to which they are to be united. The brass, as indicated in Fig. 20 6, may be fed in from one side either by hand or automatic means, as desired.

With either of the foregoing forms of apparatus it is rendered possible to rapidly assemble a large number of bonds and terminal pieces in properly aligned position and the brazing of the two together may thereupon be accomplished with expedition and assurance that a uniformly perfect junction is secured in each instance.

30 Other modes of applying the principle of my invention may be employed instead of the one explained, change being made as regards the means and the steps herein disclosed, provided those stated by any one of 35 the following claims or their equivalents be employed.

I therefore particularly point out and distinctly claim as my invention:—

1. The method of making a rail-bond of 40 the character described, as a separate article of manufacture, which consists in inserting the end of a conductor in a recess in a suitable mold, also placing in such recess adjacent such conductor-end a piece of metal, 45 and then heating such mold and introducing a quantity of braze in such recess, the temperature of the mold being sufficient to melt such braze whereby such conductor-end and piece of metal are firmly united together.
- 50 2. The method of making a rail-bond of the character described, as a separate article of manufacture, which consists in press-fitting a sleeve around the end of a stranded conductor, inserting such conductor-end in 55 a recess in a suitable mold, also placing in such recess adjacent such conductor-end a piece of steel, and then highly heating such mold and simultaneously introducing a quantity of braze in such recess, the temperature of the mold being sufficient to melt 60 such braze whereby such conductor-end and piece of steel are firmly united together.
- 65 3. The method of making a rail-bond of the character described, as a separate article of manufacture, which consists in press-

fitting a sleeve of the same metal around the end of a stranded copper conductor, inserting such conductor-end in a recess in a suitable mold, also placing in such recess adjacent such conductor-end a piece of steel, 70 and then highly heating such mold and introducing a quantity of braze in such recess, the temperature of the mold being sufficient to melt such braze whereby such conductor-end and piece of steel are firmly united together. 75

4. In apparatus of the character described, the combination of a recessed mold adapted to receive and hold in adjacent relation the end of a conductor and a supplemental piece 80 of metal to be attached thereto, means apart from said mold adapted to support such conductor in position with one end thereof thus held in said mold, and means for heating said mold. 85

5. In apparatus of the character described, the combination of a recessed mold adapted to receive and hold in adjacent relation the end of a conductor and a supplemental piece 90 of metal to be attached thereto, means apart from said mold adapted to support such conductor in approximately vertical position with one end thereof thus held in said mold, means for supplying braze material to said mold, and means for heating said mold. 95

6. In apparatus of the character described, the combination of a recessed mold adapted to receive and hold in adjacent relation the end of a conductor and a supplemental piece 100 of metal to be attached thereto, means apart from said mold adapted to support such conductor in position with one end thereof thus held in said mold, means for supplying braze material to said mold, and electric resistance means for heating said mold. 105

7. In apparatus of the character described, the combination of a plurality of recessed molds arranged side by side, electric resistance plates interposed between successive molds, each of the latter being adapted to 110 receive and hold in adjacent relation the end of a conductor and a supplemental piece of metal to be attached thereto, and means for passing a heating electric current through said series of molds and interposed 115 resistance plates.

8. In apparatus of the character described, the combination of a plurality of recessed molds arranged side by side, electric resistance plates interposed between successive 120 molds, each of the latter being adapted to receive and hold in adjacent relation the end of a conductor and a supplemental piece of metal to be attached thereto, means for adjustably clamping together said series of molds and interposed resistance plates, and electrodes for supplying current connected with the terminal members of said series. 125

9. In apparatus of the character described, the combination of a plurality of recessed 130

graphite molds arranged side by side, electric resistance plates interposed between successive molds, each of the latter being adapted to receive and hold in adjacent relation the end of a conductor and a supplemental piece of metal to be attached thereto, means adapted to retain a plurality of such conductors in position with the ends thereof

thus held in said molds, means for adjustably clamping together said series of molds and interposed resistance plates, and electrodes for supplying current connected with the terminal members of said series. 10

Signed by me this 16th day of January 1921.

CHARLES A. CADWELL.